

## UNITED STATES PATENT OFFICE.

ADOLPHE H. NEY, OF NEW YORK, N. Y.

## PROCESS FOR FLOTATION OF ORES.

No Drawing.

Application filed May 2, 1927. Serial No. 188,397.

This invention relates to a new and improved process for the concentration of ores by the method known as "froth flotation" and particularly to the use and employment 5 in said ore concentration process, of chemicals and substances and transformation products thereof, hitherto unknown as being of advantage or utility as agents or assisting and auxiliary substances in said ore concentration 10 process as customarily practiced.

The process of concentrating ore, commonly designated "froth flotation" consists in producing by suitable means upon the surface of an aqueous suspension of a finely comminuted 15 ore body, a froth. Under suitable conditions, this froth carries to the surface of the liquid, a "concentrate" containing a higher percentage of the metallic or other valuable constituents of the ore treated than it originally contained. This "concentrate" is continuously or 20 intermittently removed and further treated to recover and purify its valuable constituents.

A variety of substances has been hitherto 25 proposed and employed as agents or assisting and auxiliary media for producing the "concentrating effect", or as they are called "promoters" and many of these substances are indeed effective in a greater or lesser degree in that their addition to or presence in 30 the operation of flotation produces or effects the formation of a concentrate containing a higher percentage of the valuable constituents of the ore than the latter originally contained. The relative value of such flotation 35 agents also depends on the amount necessary to be effective, and the time required to produce such effect, and their price.

Examples of such "promoters" are, for instance, the products of the reaction of an 40 excess of disulphurdichloride upon certain aromatic amines, and which have the probable constitution:



45

R being a substituted aryl radical. These products may be considered as the intramolecular anhydrides, or sultams, of a substituted thiosulphanic acid: R.S.SO.OH., R being an aryl radical, substituted in the ortho- 50 position by the amino group.

I have discovered that a group of com-

pounds closely related structurally to the above and hitherto not employed or proposed for this purpose are very efficient flotation agents. These compounds are derivatives of thiosulphuric acid: HS.SO<sub>2</sub>.OH—or its salts: MES.SO<sub>2</sub>.OMe, in which the hydrogen or metal-atom of the sulphhydrate group: SH 55 (SMe) is substituted by an organic radical. The prototype of this group, sodiummethylthiosulphate: C<sub>2</sub>H<sub>5</sub>.S.SO<sub>2</sub>.ONa, has been discovered and described by Bunte, Berichte der deutschen chemischen gesellschaft, 7, (1874), 60 646 and he as well as later investigators have prepared and described other members of this group, such as n-propyl-, iso-butyl-, amyl-thiosulphate, as well as benzylthiosulphate. Compare: ber. 7 (1874) 1162; (Spring).—15. 65 (1882). 1938; (Spring and Legros).—25. (1892). 988; 26 (1893) 993.996; (Otto and Rossing).—41 (1908) 1650; (A. Gutmann); 42 (1909) 228; (A. Gutmann).—Trans. 70 Chem. Soc. 91 (1907) 2021; 93 (1909). 1395, 75 1401; (Price and Slater).—Gazz. Chim. It. 20, (1890). 25 (Purgatti).

Representatives of these groups of compounds may be prepared by allowing an alkyl- or arylalkyl-halide, such as ethylbromide or benzylchloride to react upon sodiumthiosulphate in aqueous or aqueous-alcoholic solution at temperatures from 30° C. to 100° C. In place of the halides the corresponding sulphates, as for example, sodiumethylsulphate or diethylsulphate may be used with equal success; also, the alkyl- and aryl-alkyl-radicals may be substituted with other groups such as the hydroxy-, alkyloxy-, carboxy-, sulpho-, amido-, cyan-, etc., group. If 80 the alkyl group is substituted by a further negative group, such as halogen, it is possible, according to the conditions employed, to replace either one or both of the negative groups by the thiosulphuric-rest, as for instance with 85 ethylendibromide both:



may be obtained without difficulty.

By allowing an organic acidhalide, such as benzoylchloride, acetylchloride, etc., to react in an analogous manner with sodiumthiosulphate, analogous compounds possessing similar properties may be obtained. They possess the constitution: R.C.O.S.SO<sub>2</sub>.ONa. R 10 11

indicating an alkyl, aryl or arylalkyl group, which may be substituted.—dihalides of dibasic acid, such as oxalyldibromide, also react with sodiumthiosulphate forming, under suitable conditions, compounds containing the thiosulphuric acid rest once or twice respectively.

By reacting the chlorides of organic sulphonnic acids, for example paratoluosulphochloride with sodiumthiosulphate, bodies of similar properties having the probable constitution:  $R.SO_2.SSO_2.ONa$  can be obtained.

Aromatic—or purely aromatic—analoga of these compounds:  $R.SSO_2.ONa$  and  $NaO.SO_2$ ,  $S.R.SO_2.ONa$ , in which  $R$  a substituted aryl-group can also be obtained although by different reactions. Negatively substituted cyclic hydrocarbons such as chlorbenzol, do not react with sodiumthiosulphate barring certain exceptions.—Aromatic compounds capable of assuming, or possessing, quinoid character, however, as a rule, smoothly react with thiosulphate under formation of substituted aromatic thiosulphates of the type:



where  $X$  may be hydrogen or alkyl. Compare: Bernthsen, Ann. 251.50; Green, British Patent. 4792 of 1900.

Similarly, benzoquinons, hydroquinons and their substitution products, especially chlor-substitution products react under suitable conditions with one or several molecules of sodiumthiosulphate under formation of hydroquinone-monothiosulphate, hydroquinone-di-thiosulphate and hydroquinone-tetra-thiosulphate, which on oxidation yield the corresponding quinonemono or polythiosulphonic acid, or the corresponding di- or polysulphides. Compare: German Patent. 175070.

These compounds are, in form of their alkali salts, in general, well crystallizing bodies, easily soluble in water and, though less readily, in alcohol. Under the influence of reducing agents, or even under the influence of hydrolyzing agents, such as diluted mineral acid at the boil, they are transformed into the corresponding thiophenols, while upon treatment with oxidizing agents, they yield according to the nature of the oxidizing agent used and the experimental conditions di- or polysulphides, presumably, for instance, according to the following equation:



$R$  being alkyl, arylalkyl or acyl- rest, which may be substituted.—The solubility of these compounds in water decreases with the increase of their molecular weight, as does their stability, evidenced by an increased tendency to conversion into disulphidic form.

I have prepared a considerable number of members of this class of compounds, for ex-

ample: sodiummethyl-, sodiumethyl-, sodium-n-propyl-, sodium-iso-propyl-, sodium-iso-butyl- and sodium-iso-amyl-thiosulphate, by the reaction of the corresponding alkyl-halids or alkylsulphates upon thiosulphate, 70 in several instances by both methods, and I have prepared benzylthiosulphate from benzylchloride and thiosulphate; I have also prepared the reaction products of sodiumthiosulphate with the following compounds: chloro- 75 acetic acid, glycerolmonochlorhydrine, glycerolmonochlorhydrine, glyceroldichlorhydrine, ethylendichloride (both one and both chlorine-atoms replaced by the thiosulphate rest), benzolsulphochloride, paratoluolsulphochloride 80 and malonylchloride. When subjected to flotation tests all these compounds were found to be excellent "promoters", particularly sodiummethylthiosulphate, sodium-isopropylthiosulphate, sodium-isobutylthiosulphate 85 and sodiumbenzylthiosulphate.

To illustrate the use of these compounds the following example is given:

*Example.*

90

600 grs. of a sulphidic copper bearing ore containing 1.2% copper were ground to fineness of #60 mesh with some water, 5 grs. slaked lime and 0.25 grs. sodium-ethyl-thiosulphate added and the mixture transferred 95 to a flotation cell, diluted and aeration started. Pine oil was added in drops as needed to produce frothing and the froth removed at intervals. Aeration was continued for 30 minutes, whereupon the collected froth was 100 filtered and dried. It weighed, when dry, 67 grs. and contained 10% of copper; an extraction of 93.2% of the copper present having thus been effected.

When replacing in parallel tests the sodium-ethyl-thiosulphate by similar amounts of sodium-isopropylthiosulphate, sodium-isobutylthiosulphate and sodium-benzylthiosulphate, results very closely approximating that described above were obtained.

110

It is understood that my invention is not limited to the proportions of materials given nor to the nature of subsidiary agents employed. Neither do I wish to be restricted to the use of any particular method or modus 111 of working or operation, or to any particular type of apparatus or machinery, all these things being capable of variation and modification according to the nature of the ore treated and the result desired. It is further 120 to be understood that my invention is not limited to the compounds specifically mentioned herein, nor to those which I have actually examined as to their efficiency as flotation agents—viz: 27 different compounds of 121 this class—but I wish it expressly to be understood that my invention includes all and any compounds which are derivatives of thiosulphuric acid or its salts obtainable from it by replacement of the hydrogen or metal- 130

atom of the sulphhydrate group by an organic radical, such compounds having the constitution:

5



R being an organic radical, which may be substituted and may contain the thiosulphate 10 rest a second time or more times.

Their general efficiency as "promoters" in ore flotation appears to be—and probably is—due in part to their tendency to assume under oxidative influences, disulphidic form.

15 When employing these compounds as flotation agents, it is not necessary that they be pure; excellent results, for instance, are obtained when the crude mixture obtained from the reaction of one molecule of sodium 20 thiosulphate and  $\frac{1}{2}$  molecule of diethylsulphate, consisting of approximately 70% sodiummethylthiosulphate and 30% sodiumsulphate, is used as flotation agent. It is evident that this point is of great importance in regard to the economy of the process, and cost 25 of material.

Having thus described the nature of my said invention and in what manner it may be applied, I declare that what I claim is:

1. The method of concentrating ores by 30 froth flotation which includes subjecting the crushed mineral to a froth floating process in the presence of a derivative of thiosulphuric acid, in which the hydrogen atom of the sulphhydrate group is replaced by an 35 alkyl group.

2. The method of concentrating ores by froth flotation which comprises subjecting the mineral in form of an alkaline pulp to a froth flotation operation in the presence of 40 sodiumalkylthiosulphate and a suitable frothing agent.

3. The method of concentrating ores by froth flotation which comprises subjecting the mineral in the form of a pulp rendered 45 alkaline with lime to a froth flotation operation in the presence of sodiumalkylthiosulphate and a suitable frothing agent.

In testimony whereof I affix my signature.

ADOLPHE H. NEY.